

# UNITED STATES PATENT OFFICE.

ERNST THALMANN, OF WINTERTHUR, SWITZERLAND.

## MATERIAL FOR CLEANING THE TYPES OF PRINTING APPARATUS AND PROCESS FOR ITS PREPARATION.

No Drawing. Application filed October 10, 1922, Serial No. 593,627, and in Switzerland April 3, 1922.

The subject of the present invention is a material for cleansing the types of printing apparatuses, such for instance, as type writing machines, cash registers or stamps, by a dry process by aid of dabbing, and a process for its preparation.

The material consists of a plastic mass by means of which the types are dabbed and which can be prepared in the following manner, (by way of example). A plastic compound containing clay and glycerine, and, if desired, a suitable coloring matter, is mixed with a predetermined quantity of colophonium and petroleum. Such a compound may be prepared by mixing together clay and glycerine in the approximate proportions of 40 parts and 10 parts by weight respectively and adding thereto approximately 10 parts by weight of a concentrated solution of colophonium in crude petroleum. A mixture of pulverized Pará rubber and talc in approximately equal parts by weight is then prepared, and 30-40 parts by weight of this mixture is mixed with 60-70 parts by weight of the first mixture. To the mass thus obtained is then added pure glycerine and a small quantity of a solution of resin, preferably in the form of a slimy semi-fluid mass, gamboge having been found to be a suitable form of resin for this purpose, and the preferred solvent being petroleum. The entire mixture is then pressed and heated, after which it is rolled between heated rollers until it is reduced to a very fine, homogeneous plastic mass, which is then preferably pressed into strands, from which plugs of convenient size are cut. The cleansing mass thus prepared is very permanent. It does not become hard, but retains its plasticity for a very long time, and a plug can, after use, be rendered suitable for re-use by kneading it, and this may continue for months.

The application of the material consists in pressing the mass upon the types and immediately removing such mass (dabbing), whereby the dirt is taken up by the mass leaving the types clean again.

The dirty part of the mass is preferably each time folded inwards and in this manner one plug can be utilized for a long period without loss of material and without losing its effect.

Having now particularly described and ascertained the nature of my said invention and in what manner the same is to be performed, I declare that what I claim and desire to secure by Letters Patent of the United States is:—

1. A cleansing compound for the type of printing apparatus comprising a plastic mass containing a mixture of clay, glycerine, colophonium, petroleum, Pará rubber, talc, and resin.

2. A cleansing compound for the type of printing apparatus, comprising a plastic mass containing a mixture of clay, glycerine, colophonium and petroleum, and a mixture of Pará rubber, resin and talc, the proportion of the first mixture being approximately 60 to 70 by weight and that of the second mixture approximately 30 to 40 by weight.

3. The process of manufacturing a cleansing compound for the type of printing apparatus, which consists in mixing together a plastic compound containing clay, glycerine, colophonium and petroleum, adding thereto a mixture of pulverized rubber and talc, adding glycerine and a solution of resin, pressing and heating the mass, and rolling the same into a homogeneous, plastic mass.

In testimony whereof I have signed my name to this specification.

ERNST THALMANN.